# EUROPEAN PATENT APPLICATION

(11) **EP 0 382 159 A1**
(43) Date of publication of application: **16.08.1990**
(21) Application number: 90102296.2
(22) Date of filing: 06.02.1990
(51) Int. Cl.: C10L 1/18, C10L 10/04

(54) **Defouling of fuel systems**

(30) Priority: 06.02.1989 US 306575
(71) Applicant: E.I. DU PONT DE NEMOURS AND COMPANY, Wilmington Delaware 19898 (US)
(72) Inventor: Smiley, Robert Arthur, Wilmington, Delaware 19803 (US)
(74) Representative: Abitz, Walter, Dr.-Ing.

(57) **Abstract**

Dibasic esters of C₄ to C₆ aliphatic acids when added to the fuel induction system of an internal combustion engine effectively remove deposits and restore better performance.

## Description

### Field of the Invention

This invention relates to a method for cleaning the carburetor and associated fuel induction and combustion parts of an internal combustion engine, to a method for cleaning the fuel induction system of an internal combustion engine having fuel injectors, and to a hydrocarbon fuel for an internal combustion engine containing at least one member of a particular class of deposit removing and residue inhibiting compounds.

### Background of the Invention

Unsatisfactory operation of both carbureted and fuel injection gasoline engines occurs when gum and varnish deposits build up in their fuel systems. A major cause of such deposits is the recycling of blowby gases from the crankcase to the air intake supply. Such deposits plug carburetor jets and fuel injector nozzles, preventing proper fuel flow. Also, deposits may coat intake valves or spark plug electrodes, interfering with efficient fuel combustion.

It is desirable for efficient engine performance to remove the deposits formed in the carburetor and fuel injectors as well as in their associated fuel system components. In carbureted fuel systems, a method that has been used to clean away the deposits is to slowly pour or spray a solvent through the mouth of the carburetor while the engine is running. Solvents and their mixtures that have been used in this way include methanol, petroleum distillates, xylenes, diacetone alcohol, and 2-butoxyethanol. Their use has met with only limited success since their cleaning effectiveness is limited to the cooler parts of the system. They do not dissolve or remove many of the varnish deposits and when added to the carburetor, their vapors usually stop or "kill" the engine.

Another procedure used to effect contact between a cleaning composition and the undesirable deposits in a carburetor is to add the cleaning agent to the fuel. This approach is necessary for fuel injector systems since there is no convenient method to directly contact the injector with the cleaning composition as there is in a carburetor. By this procedure, the cleaning compositions, often referred to as detergents, contact the fuel injector or carburetor deposits as they are carried in their solution in gasoline through the fuel system. Such detergents, although they may clean the carburetor or fuel injectors, often decompose in the hotter parts of the engine, such as at the valves, to form deposits, thus increasing octane requirements. Various detergents have been added to hydrocarbon fuels to reduce the extent of such deposits. See for example Kuhn, U.S. Patent 4,072,474. Noke, U.S. Patent 4,004,894, and Vas, U.S. Patent 4,728,340.

It is an object of this invention to provide a process which not only cleans carburetors and fuel injectors of undesirable deposits, but cleans the remainder of the fuel induction system including the valves and ports. This process involves the use of a solvent composition containing at least 20% of a principal component which is a C₁-C₄ alkyl diester of one or more C₄-C₆ aliphatic dibasic acids, particularly succinic, glutaric, and adipic acids. Other components of the cleaner may be a gasoline detergent, a rust inhibitor, and one or more non-halogen-containing organic solvents. A preferred C₁-C₄ dialkyl ester of C₄-C₆ aliphatic dibasic acids is a mixture by weight of 15-25% dimethyl succinate, 55-75% dimethyl glutarate and 10-25% dimethyl adipate. Its approximate boiling range is 196-225°C, and its vapor pressure at 20°C is 0.2 Torr. A second preferred dibasic ester component is dimethyl adipate containing 0-15% by weight dimethyl glutarate.

The effectiveness of the dibasic ester solvent in cleaning fuel systems is believed to be a result of ts excellent solvency combined with its high boiling temperature and excellent thermal stability. For example, when added through the carburetor throat, the dibasic ester solvent stays liquid going through the venturi section and wets and cleans the throttle plate and body. It also flows down and wets and cleans the intake valves. With a manifold gage, an increase in vacuum is observed after a dibasic ester solvent treatment.

### Summary of the Invention

The present invention is a process for the cleaning of a carburetor and accompanying fuel induction parts used as engine valves parts, as well as spark plugs and the cylinder walls of the engine. This process comprises adding an effective amount of at least one C₁ to C₄ dialkyl ester of a C₄ to C₆ aliphatic dibasic acid to the carburetor while the engine is running.

Another aspect of the present invention is cleaning the fuel injectors of an engine equipped with fuel injectors by running the engine on a fuel mixture containing 0.2 to 8 ounces of the aforementioned dialkyl ester per gallon of fuel.

Another aspect of the present invention is a hydrocarbon fuel containing 0.2 to 8 ounces of the aforementioned dialkyl ester per gallon of fuel.

### Detailed Description

The method of cleaning a fouled carburetor of an internal combustion engine comprises adding an effective amount of at least one C₁ to C₄ dialkyl ester of a C₄ to C₆ aliphatic dibasic acid to the carburetor while the engine is running. "An effective amount" will vary depending on the size of the carburetor, the speed that the engine is running and the degree to which the carburetor is fouled, but generally about 2 ounces of the aliphatic dibasic acid ester must be added before there is any noticeable change in engine performance. It is preferable to add the ester through the air intake throat of the carburetor, which is readily accessible on most engines by removal of the air filter cover or the air filter itself.

The process of cleaning a carburetor by the direct addition of cleaner to the carburetor, comprises using a composition containing at least 20% and preferably at least 40% by weight of at least one C₁ to C₄ dialkyl ester of at least one C₄ to C₆ aliphatic dibasic acid. In some situations the cleaner may be almost entirely composed of the dialkyl ester. The dialkyl ester in most cases will be a mixture of C₄ to C₆ aliphatic dibasic acid. Mixtures of C₄ to C₆ dibasic acids are a byproduct of the manufacture of adipic acid -- an acid that is used commercially on a large scale in the production of some types of nylon. Suitable dialkyl esters for use in the present invention are obtained by the esterification of such a byproduct stream. The composition of such a byproduct stream varies considerably, but in general will contain about 15 to 30 percent succinic acid, 50 to 73 percent glutaric acid, and about 6 to 25 percent adipic acid. The methyl esters of such a mixture of acids are usually the most economically attractive, but ethyl, propyl and butyl esters are also useful.

Another major, but optional component in the cleaner is one or more non-halogen-containing organic solvents preferably those that have high flash points, i.e., above about 140°F. Such solvents include N-methyl-2-pyrrolidone, esters of monoalkyl ethers of dipropylene glycol, and esters of monoalkyl ethers of tripropylene glycol, and blends of hydrocarbons sometimes called "heavy aromatic naptha".

Other components that may be included are conventional gasoline detergents and rust inhibitors.

The hydrocarbon fuel of the invention comprises the fuel component, i.e, the petroleum fraction with or without the conventional additives, and about 0.2 to about 8 ounces per gallon of at least one C₁ to C₄ dialkyl ester of a C₄ to C₆ aliphatic dibasic acid.

The method of cleaning a fuel system of an internal combustion engine having fuel injectors is running the engine on the above described hydrocarbon fuel containing the aliphatic dibasic acid ester in the amounts set forth. An engine with partially plugged fuel injectors will normally run noticeably better after about 1/4 to 1/2 tank of fuel containing the ester is burned. It is not necessary to run the engine at any particular speed to obtain the improvement -- merely adding the required amount of ester to the gas tank and using the engine in its usual fashion will yield the improvement.

### Example 1

A 302 V/8 Ford engine was modified by replacing the standard carburetor air system by a "Y" manifold. Each arm of the manifold was fitted with a single barrel carburetor. Each carburetor was fitted with a removable aluminum sleeve in the area of the throttle plate in the carburetor base. Below the carburetor in each intake manifold was mounted a removable heated deposit tube fitted with a thermocouple. The engine test conditions were as follows:
Engine RPM's: 700 + or - 50
Inlet air temperature: 160°F + or - 5
Intake deposit bar temperature: 275°F + or - 5
Base fuel: Phillips J gasoline

The engine was run for about 15 hours using the base fuel, which is known to form deposits. The "dirty" sleeves and deposit tubes were removed, weighed, and replaced. The engine was restarted, 4 oz. a mixture of dibasic esters (about 17% by wt dimethyl succinate, about 66% by wt dimethyl glutarate, and about 17% by wt dimethyl adipate) was poured through carburetor #2. Nothing was added to carburetor #1. The engine was run for 60 minutes following the addition. The sleeves and deposit tubes were removed and weighed. The results were:

| | Deposit Weight, mg. |
|---|---|
| Sleeve carburetor #1, dirty, 15 hr. | 3.0 |
| Sleeve carburetor #1, (1 hr. later) | 2.9 |
| Sleeve carburetor #2, dirty, 15 hr. | 3.0 |
| Sleeve carburetor #2, (Treated + 1 hr.) | 0.0 |
| Deposit tube #1, dirty, 15 hr. | 14.4 |
| Deposit tube #1, 1 hr. later | 9.0 |
| Deposit tube #2, dirty, 15 hr. | 15.7 |
| Deposit tube #2, treated + 1 hr. | 1.9 |

The above results show that the dibasic ester treatment effectively removed deposits both from the sleeve in the area of the carburetor base and from the heated tube in the intake manifold.

### Example 2

A 1985 Oldsmobile Cutlass Ciero fitted with a 3.8 liter V-6 engine was running poorly, i.e. it hesitated and appeared to be operating on less than six cylinders. The probable cause of this poor performance was diagnosed as one or more clogged fuel injectors. When the fuel gage read one eighth full (approximately 2 gal), a pint of a mixture of dibasic esters (about 18% by wt dimethyl succinate, about 65% by wt dimethyl glutarate, and about 17% dimethyl adipate) was added to the fuel tank. The car was started and allowed to run at idle speed for 20 min. The engine was turned off and after an hour of not running, the gas tank was filled to capacity and the car restarted and tested by driving at normal highway speed. The hesitation was gone and the car ran at high efficiency demonstrating that the fuel injectors had been unclogged by the dibasic ester treatment.

## Claims

1. A method of cleaning the carburetor of an internal combustion engine which comprises adding an effective amount of at least one C₁ to C₄ dialkyl ester of a C₄ to C₆ aliphatic dibasic acid to the carburetor of the engine while the engine is running.

2. The method of claim 1 in which a mixture of dialkyl esters of dibasic acids is added to the carburetor.

3. The method of claim 2 in which the mixture contains 15 to 25% dimethyl succinate, 55 to 75% dimethyl glutarate, and 10 to 25% dimethyl adipate.

4. The method of claim 2 in which the rate of addition of the dialkyl ester of dibasic acids is such that the engine speed is not significantly changed, and in which the amount of dialkyl ester of dibasic acids added is at least 2 ounces.

5. A method of cleaning the fuel system of an internal combustion engine having fuel injectors which comprises running the engine on a fuel mixture containing about 0.2 to about 8 ounces of at least one C₁ to C₄ dialkyl ester of a C₄ to C₆ aliphatic dibasic acid per gallon of fuel.

6. A liquid hydrocarbon fuel for an internal combustion engine containing a deposit removing and residue inhibiting amount of at least one C₁ to C₄ dialkyl ester of a C₄ to C₆ aliphatic dibasic acid.

7. The hydrocarbon fuel of claim 6 in which the amount of aliphatic dibasic acid ester is between about 0.2 ounces and about 8 ounces per gallon of fuel.

8. The hydrocarbon fuel of claim 6 in which contains a mixture of dialkyl aliphatic dibasic esters.

9. The hydrocarbon fuel mixture of claim 8 in which the mixture of dialkyl aliphatic dibasic esters are dimethyl esters of glutaric, succinic, and adipic acid.
